

# UNITED STATES PATENT OFFICE.

ROBERT W. HULL, OF HINGHAM, MASSACHUSETTS.

## REFRACTORY MATERIAL AND PROCESS OF MAKING SAME.

1,418,648.

Specification of Letters Patent. Patented June 6, 1922.

No Drawing.

Application filed April 9, 1921. Serial No. 459,999.

To all whom it may concern:

Be it known that I, ROBERT W. HULL, a citizen of the United States of America, and a resident of Hingham, in the county of 5 Plymouth and State of Massachusetts, have invented certain new and useful Improvements in Refractory Materials and Processes of Making Same, of which the following is a specification.

10 This invention relates to refractory material to be used as a lining for surfaces subjected to intense heat and it has for its object the production of a material of this character composed of the tailings of a concentrating 15 mill in which disseminated chrome ore has been treated.

The invention consists in taking the waste material left in concentrating disseminated chrome ore and grinding and mixing the 20 same and then uniting the mixture by a suitable binding material.

25 The invention further consists in subjecting said mixture to pressure and forming bricks of the compressed material.

For the purpose of describing the invention one preferred form is described, this 30 form having been found to give satisfactory and reliable results, although it is to be understood that the various elements of the combination can be variously combined, and the invention is not limited to the precise 35 combination of elements as herein described except as required by the scope of the appended claims.

When disseminated chrome ore has been 40 concentrated in a suitable mill, the "tailings" or waste material therefrom has heretofore had no commercial value.

It has been found, however, that these 45 "tailings" contain about five per cent chromite, combined with quantities of silica, serpentine, olivin, magnesite, and alumina, and these elements when united by a suitable binder make an excellent refractory material 50 particularly adapted to be used for linings of furnaces and other walls subjected to an intense heat.

The "tailings" or waste material from the 55 concentrators are ground into pulverized form, thoroughly mixed together, and then the entire mass has a binding material mixed therewith.

Portions thereof are then subjected to pressure and formed into bricks or bri- 55 quettes of such shape and size as to make

them available in the construction of furnace walls.

These bricks or briquettes are then baked in any usual manner and are ready for the market.

60 Chromite has been used heretofore in the manufacture of refractory material but in very large proportions relatively to the other elements used in said material.

In the present invention the proportion of 65 chromite used is very small and yet when combined with larger proportions of such elements as silica, serpentine, olivin, magnesite and alumina, a refractory material is produced capable of withstanding the most 70 intense heat.

The chromite, viz: iron oxid and chromic 75 oxid, remaining in the "tailings" from the concentrator form only about five per cent of the ingredients used in the manufacture of the refractory material but this proportion has been found quite sufficient to produce a most satisfactory material when combined with such ingredients as silica, serpentine, olivin, magnesite and alumina.

80 One reason why chromite is not more generally used in the manufacture of refractory materials is because it has so much greater value in other industrial arts as to make its use prohibitive.

In the present invention, it has been found possible to manufacture the refractory material with that portion of chromite which is useless in other industrial arts and which would be wasted unless utilized 90 in some such manner as is herein described.

In carrying out the manufacture of the invention, the waste material from the concentrator containing chromite, silica, alumina, serpentine, olivin, and magnesite, is pulverized and thoroughly mixed and then a suitable binding material is added thereto.

95 This mixture is then formed into desired shapes, under pressure, and baked.

The preferred mixture consists of about 100 five parts chromite and ninety-five parts of silica, alumina, serpentine, olivin, magnesite and binding material.

105 The binding material used may be pitch, tar, or any other substance suitable for such use and the quantities of silica, alumina, serpentine, olivin and magnesite may be used in any desired proportions.

During the baking of the mixed ingredients, the binding material is so acted upon 110

as to leave a residue of carbon which thoroughly unites the other ingredients and effectually prevents their separation.

When the ingredients, after mixture, are formed into bricks or briquettes and then baked, the chromite so unites with the other ingredients as to form a hardened exterior surface adapted to resist the most intense heat.

10 While for the best results it is preferred to use all the other ingredients combined with the chromite, it is obvious that good results may be obtained with one or more of these ingredients omitted.

15 The finished article will resist the highest temperature.

It is believed that the operation and many advantages of the invention will be understood readily by reference to the description 20 and to the claims to be hereinafter given.

Having thus described my invention, I claim:

1. A refractory material for surfaces subjected to intense heat comprising waste 25 material left after concentrating disseminated chrome ore containing a mixture of silica, serpentine and olivin and united by a binder.

2. A refractory material for surfaces subjected to intense heat comprising a mixture of silica, serpentine, olivin, magnesite, and alumina forming about ninety-five per cent of the compound and having mixed therewith and bonded thereto five per cent of chromite.

3. A refractory material for surfaces subjected to intense heat comprising a mixture of silica, serpentine, olivin, and magnesite

forming about ninety-five per cent of the compound and having mixed therewith and bonded thereto five per cent of chromite.

4. A refractory material for surfaces subjected to intense heat comprising a mixture of silica, serpentine and olivin forming about ninety-five per cent of the compound 45 and having mixed therewith and bonded thereto five per cent of chromite.

5. The process of making refractory material which consists in taking waste material from concentrators containing 50 chromite, magnesite, silica, olivin, serpentine, and alumina; grinding and mixing the same; and then adding a binding material thereto.

6. The process of making refractory material which consists in taking waste material from concentrators containing chromite, magnesite, silica, olivin, serpentine, and alumina; grinding and mixing the same; adding a binding material thereto; 60 subjecting the material to pressure to form it into a desired shape; and then baking the same.

7. The process of making refractory material which consists in mixing about 65 five per cent of chromite with a mixture containing about ninety-five per cent of ingredients of a crystalline nature; grinding the same; and adding a binding material thereto.

Signed by me at 294 Washington St., Boston, Mass., this 7th day of April, 1921.

ROBERT W. HULL.

Witnesses:

WALTER E. LOMBARD,  
NATHAN C. LOMBARD.